

May 22, 1962

E. D. BOLINGER

3,035,328

METHOD OF PREPARING CRIMPED YARNS

Original Filed Nov. 2, 1955



FIG. -1-



FIG. -2-

INVENTOR.  
EDGAR DARE BOLINGER  
BY *Roger R. Jones*  
ATTORNEY

**1**

3,035,328

**METHOD OF PREPARING CRIMPED YARNS**  
Edgar Dare Bolinger, Clemson, S.C., assignor to Deering  
Milliken Research Corporation, near Pendleton, S.C.,  
a corporation of Delaware  
Original application Nov. 2, 1955, Ser. No. 544,521, now  
Patent No. 2,919,534, dated Jan. 5, 1960. Divided  
and this application Mar. 2, 1959, Ser. No. 796,423  
7 Claims. (Cl. 28—72)

This invention relates to methods for producing fabrics and yarns having an elastic nature and is a division of U.S. application Serial Number 544,521, filed November 2, 1955, now U.S. Patent 2,919,534, and a continuation-in-part of application Serial Number 274,358, filed March 1, 1952.

A number of methods for producing fabrics and yarns which have an elastic nature are now well known in the art. For example, it is known that a thermoplastic yarn having an elastic nature can be produced by twisting an uncrimped, continuous filament thermoplastic yarn, heat setting the highly twisted yarn, and thereafter untwisting, and it is also known that a yarn having an elastic nature can be produced by passing a thermoplastic yarn into a heated stuffing box or between heated intermeshing gear wheels. However, such prior art methods are not satisfactory in all respects since either the yarn has an inadequate degree of elasticity or else the yarn is so highly crimped that handling of the same, for example during weaving and knitting operations, is difficult.

It is an object of the invention to provide methods for the production of yarns which tend to assume a highly convoluted configuration which are not subject to the disadvantages of prior art processes and to methods for processing yarns free of torsional stresses but containing latent differential longitudinal stresses.

Yarns free of torsional stresses but containing latent differential longitudinal stresses can be produced by passing a thermoplastic yarn under tension from a source of supply along a linear path having a curved portion providing an abrupt change of direction, followed immediately by a portion having a lesser amount of curvature i.e., having a relatively great radius of curvature or a straight line path which can be regarded as having an infinite radius of curvature. The yarn is heated so that at least during its passage through the curved portion of the path it is at an elevated temperature but preferably is allowed to cool during its passage through the curved portion of the path having a relatively large radius of curvature. After being allowed to cool under tension, the latent differential longitudinal stresses in the yarn are released by reheating the yarn under such conditions as to permit it to assume a distorted linear configuration, and this second heating operation fully develops the elastic nature of the yarn.

The yarn, subsequent to passage through the angular course but before the second heating operation, is herein-after referred to as "latentely" elasticized yarn, since, as explained above, it is not until after the second heating operation that the yarn develops its full elastic nature. The filaments in the latentely elasticized yarn are characterized by a slightly wavy or coiled appearance when in an untensioned condition and in most instances have a slightly flattened cross section. The linear distortions or coils are generally relatively small in number, occurring in some instances as infrequently as 5 or 6 per inch, and are generally of a relatively large amplitude, having diameters of from about 1 to 3 millimeters in the case of filaments smaller than about 30 denier. For example, in a 15 denier monofilament nylon yarn the loops were found to have an average diameter of 1.85 mm. and in the case of a 70 denier, 34 filament nylon yarn the loops were found to

**2**

have an average diameter of 1.58 millimeters. The loops are generally of random sizes but on occasion yarn will be found in which all of the loops appear to be of a substantially constant size. Where the yarn is composed of 5 a plurality of filaments, the loops in adjacent filaments will frequently be found to be running in opposite directions so that the yarn is very bulky in nature.

It is a feature of the invention that if the starting yarn is free of torsional stresses and if no torsional stresses are 10 deliberately introduced during processing, the latentely elasticized yarn will be substantially free of torsional stresses and only localized torsional stresses resulting from loop or coil formation will be present when in either a tensioned or untensioned condition. The loops or coils are 15 formed such that about 50% of the loops in each filaments are in one direction and the remaining half of the loops are in the opposite direction so that there is no overall tendency for the yarn to twist when the loops are removed by tensioning the yarn. This does not mean, however, 20 that there is a reversal point between each individual loop, but to the contrary the yarn will generally carry several adjacent loops running in one direction before a reversal point is encountered, and in some instances the loops will run in the same direction for as much as several inches before reversing their direction. Latently elasticized yarns according to this invention are, however, characterized by approximately 50% of the loops in each filament running in one direction and 50% in the other only when the filaments are retained substantially free of torsional stresses, 25 and if the yarn is twisted prior to processing or if torsional stresses are deliberately introduced during processing, the loops will form in a manner to largely relieve these stresses. In other words, by employing a twisted monofilament yarn as a starting material, or by twisting the 30 35 yarn during processing, a latently elasticized yarn having the loops all running in the same direction can readily be prepared. Of course, as will be apparent to those skilled in the art, the torsional stresses in such instances are reintroduced when the coils in the yarn are removed under tension so that a twisted yarn should not be employed where torsional stresses are objectionable after weaving or knitting.

The appearance of the yarn in its final form depends upon a number of factors including the conditions under 40 45 which the second heating operation is performed. If the latently elasticized yarn is developed by heating a skein of the yarn in an untensioned condition, the fully elasticized yarn will be characterized by an appearance approximating that of the latently elasticized yarn except 50 that the loops or coils will be smaller in diameter and more closely spaced. If the yarn filaments are substantially free of torsional stresses in the first instance, the small loops are formed such that about 50% of the loops are in one direction and the remaining half of the loops 55 are in the opposite direction just as in the latently elasticized yarn. The groups of coils will be of random lengths and the coils will be of random pitch. If the 60 65 70 75 80 85 90 95 98 99 99.5 100 100.5 101 101.5 102 102.5 103 103.5 104 104.5 105 105.5 106 106.5 107 107.5 108 108.5 109 109.5 110 110.5 111 111.5 112 112.5 113 113.5 114 114.5 115 115.5 116 116.5 117 117.5 118 118.5 119 119.5 120 120.5 121 121.5 122 122.5 123 123.5 124 124.5 125 125.5 126 126.5 127 127.5 128 128.5 129 129.5 130 130.5 131 131.5 132 132.5 133 133.5 134 134.5 135 135.5 136 136.5 137 137.5 138 138.5 139 139.5 140 140.5 141 141.5 142 142.5 143 143.5 144 144.5 145 145.5 146 146.5 147 147.5 148 148.5 149 149.5 150 150.5 151 151.5 152 152.5 153 153.5 154 154.5 155 155.5 156 156.5 157 157.5 158 158.5 159 159.5 160 160.5 161 161.5 162 162.5 163 163.5 164 164.5 165 165.5 166 166.5 167 167.5 168 168.5 169 169.5 170 170.5 171 171.5 172 172.5 173 173.5 174 174.5 175 175.5 176 176.5 177 177.5 178 178.5 179 179.5 180 180.5 181 181.5 182 182.5 183 183.5 184 184.5 185 185.5 186 186.5 187 187.5 188 188.5 189 189.5 190 190.5 191 191.5 192 192.5 193 193.5 194 194.5 195 195.5 196 196.5 197 197.5 198 198.5 199 199.5 200 200.5 201 201.5 202 202.5 203 203.5 204 204.5 205 205.5 206 206.5 207 207.5 208 208.5 209 209.5 210 210.5 211 211.5 212 212.5 213 213.5 214 214.5 215 215.5 216 216.5 217 217.5 218 218.5 219 219.5 220 220.5 221 221.5 222 222.5 223 223.5 224 224.5 225 225.5 226 226.5 227 227.5 228 228.5 229 229.5 230 230.5 231 231.5 232 232.5 233 233.5 234 234.5 235 235.5 236 236.5 237 237.5 238 238.5 239 239.5 240 240.5 241 241.5 242 242.5 243 243.5 244 244.5 245 245.5 246 246.5 247 247.5 248 248.5 249 249.5 250 250.5 251 251.5 252 252.5 253 253.5 254 254.5 255 255.5 256 256.5 257 257.5 258 258.5 259 259.5 260 260.5 261 261.5 262 262.5 263 263.5 264 264.5 265 265.5 266 266.5 267 267.5 268 268.5 269 269.5 270 270.5 271 271.5 272 272.5 273 273.5 274 274.5 275 275.5 276 276.5 277 277.5 278 278.5 279 279.5 280 280.5 281 281.5 282 282.5 283 283.5 284 284.5 285 285.5 286 286.5 287 287.5 288 288.5 289 289.5 290 290.5 291 291.5 292 292.5 293 293.5 294 294.5 295 295.5 296 296.5 297 297.5 298 298.5 299 299.5 300 300.5 301 301.5 302 302.5 303 303.5 304 304.5 305 305.5 306 306.5 307 307.5 308 308.5 309 309.5 310 310.5 311 311.5 312 312.5 313 313.5 314 314.5 315 315.5 316 316.5 317 317.5 318 318.5 319 319.5 320 320.5 321 321.5 322 322.5 323 323.5 324 324.5 325 325.5 326 326.5 327 327.5 328 328.5 329 329.5 330 330.5 331 331.5 332 332.5 333 333.5 334 334.5 335 335.5 336 336.5 337 337.5 338 338.5 339 339.5 340 340.5 341 341.5 342 342.5 343 343.5 344 344.5 345 345.5 346 346.5 347 347.5 348 348.5 349 349.5 350 350.5 351 351.5 352 352.5 353 353.5 354 354.5 355 355.5 356 356.5 357 357.5 358 358.5 359 359.5 360 360.5 361 361.5 362 362.5 363 363.5 364 364.5 365 365.5 366 366.5 367 367.5 368 368.5 369 369.5 370 370.5 371 371.5 372 372.5 373 373.5 374 374.5 375 375.5 376 376.5 377 377.5 378 378.5 379 379.5 380 380.5 381 381.5 382 382.5 383 383.5 384 384.5 385 385.5 386 386.5 387 387.5 388 388.5 389 389.5 390 390.5 391 391.5 392 392.5 393 393.5 394 394.5 395 395.5 396 396.5 397 397.5 398 398.5 399 399.5 400 400.5 401 401.5 402 402.5 403 403.5 404 404.5 405 405.5 406 406.5 407 407.5 408 408.5 409 409.5 410 410.5 411 411.5 412 412.5 413 413.5 414 414.5 415 415.5 416 416.5 417 417.5 418 418.5 419 419.5 420 420.5 421 421.5 422 422.5 423 423.5 424 424.5 425 425.5 426 426.5 427 427.5 428 428.5 429 429.5 430 430.5 431 431.5 432 432.5 433 433.5 434 434.5 435 435.5 436 436.5 437 437.5 438 438.5 439 439.5 440 440.5 441 441.5 442 442.5 443 443.5 444 444.5 445 445.5 446 446.5 447 447.5 448 448.5 449 449.5 450 450.5 451 451.5 452 452.5 453 453.5 454 454.5 455 455.5 456 456.5 457 457.5 458 458.5 459 459.5 460 460.5 461 461.5 462 462.5 463 463.5 464 464.5 465 465.5 466 466.5 467 467.5 468 468.5 469 469.5 470 470.5 471 471.5 472 472.5 473 473.5 474 474.5 475 475.5 476 476.5 477 477.5 478 478.5 479 479.5 480 480.5 481 481.5 482 482.5 483 483.5 484 484.5 485 485.5 486 486.5 487 487.5 488 488.5 489 489.5 490 490.5 491 491.5 492 492.5 493 493.5 494 494.5 495 495.5 496 496.5 497 497.5 498 498.5 499 499.5 500 500.5 501 501.5 502 502.5 503 503.5 504 504.5 505 505.5 506 506.5 507 507.5 508 508.5 509 509.5 510 510.5 511 511.5 512 512.5 513 513.5 514 514.5 515 515.5 516 516.5 517 517.5 518 518.5 519 519.5 520 520.5 521 521.5 522 522.5 523 523.5 524 524.5 525 525.5 526 526.5 527 527.5 528 528.5 529 529.5 530 530.5 531 531.5 532 532.5 533 533.5 534 534.5 535 535.5 536 536.5 537 537.5 538 538.5 539 539.5 540 540.5 541 541.5 542 542.5 543 543.5 544 544.5 545 545.5 546 546.5 547 547.5 548 548.5 549 549.5 550 550.5 551 551.5 552 552.5 553 553.5 554 554.5 555 555.5 556 556.5 557 557.5 558 558.5 559 559.5 560 560.5 561 561.5 562 562.5 563 563.5 564 564.5 565 565.5 566 566.5 567 567.5 568 568.5 569 569.5 570 570.5 571 571.5 572 572.5 573 573.5 574 574.5 575 575.5 576 576.5 577 577.5 578 578.5 579 579.5 580 580.5 581 581.5 582 582.5 583 583.5 584 584.5 585 585.5 586 586.5 587 587.5 588 588.5 589 589.5 590 590.5 591 591.5 592 592.5 593 593.5 594 594.5 595 595.5 596 596.5 597 597.5 598 598.5 599 599.5 600 600.5 601 601.5 602 602.5 603 603.5 604 604.5 605 605.5 606 606.5 607 607.5 608 608.5 609 609.5 610 610.5 611 611.5 612 612.5 613 613.5 614 614.5 615 615.5 616 616.5 617 617.5 618 618.5 619 619.5 620 620.5 621 621.5 622 622.5 623 623.5 624 624.5 625 625.5 626 626.5 627 627.5 628 628.5 629 629.5 630 630.5 631 631.5 632 632.5 633 633.5 634 634.5 635 635.5 636 636.5 637 637.5 638 638.5 639 639.5 640 640.5 641 641.5 642 642.5 643 643.5 644 644.5 645 645.5 646 646.5 647 647.5 648 648.5 649 649.5 650 650.5 651 651.5 652 652.5 653 653.5 654 654.5 655 655.5 656 656.5 657 657.5 658 658.5 659 659.5 660 660.5 661 661.5 662 662.5 663 663.5 664 664.5 665 665.5 666 666.5 667 667.5 668 668.5 669 669.5 670 670.5 671 671.5 672 672.5 673 673.5 674 674.5 675 675.5 676 676.5 677 677.5 678 678.5 679 679.5 680 680.5 681 681.5 682 682.5 683 683.5 684 684.5 685 685.5 686 686.5 687 687.5 688 688.5 689 689.5 690 690.5 691 691.5 692 692.5 693 693.5 694 694.5 695 695.5 696 696.5 697 697.5 698 698.5 699 699.5 700 700.5 701 701.5 702 702.5 703 703.5 704 704.5 705 705.5 706 706.5 707 707.5 708 708.5 709 709.5 710 710.5 711 711.5 712 712.5 713 713.5 714 714.5 715 715.5 716 716.5 717 717.5 718 718.5 719 719.5 720 720.5 721 721.5 722 722.5 723 723.5 724 724.5 725 725.5 726 726.5 727 727.5 728 728.5 729 729.5 730 730.5 731 731.5 732 732.5 733 733.5 734 734.5 735 735.5 736 736.5 737 737.5 738 738.5 739 739.5 740 740.5 741 741.5 742 742.5 743 743.5 744 744.5 745 745.5 746 746.5 747 747.5 748 748.5 749 749.5 750 750.5 751 751.5 752 752.5 753 753.5 754 754.5 755 755.5 756 756.5 757 757.5 758 758.5 759 759.5 760 760.5 761 761.5 762 762.5 763 763.5 764 764.5 765 765.5 766 766.5 767 767.5 768 768.5 769 769.5 770 770.5 771 771.5 772 772.5 773 773.5 774 774.5 775 775.5 776 776.5 777 777.5 778 778.5 779 779.5 780 780.5 781 781.5 782 782.5 783 783.5 784 784.5 785 785.5 786 786.5 787 787.5 788 788.5 789 789.5 790 790.5 791 791.5 792 792.5 793 793.5 794 794.5 795 795.5 796 796.5 797 797.5 798 798.5 799 799.5 800 800.5 801 801.5 802 802.5 803 803.5 804 804.5 805 805.5 806 806.5 807 807.5 808 808.5 809 809.5 810 810.5 811 811.5 812 812.5 813 813.5 814 814.5 815 815.5 816 816.5 817 817.5 818 818.5 819 819.5 820 820.5 821 821.5 822 822.5 823 823.5 824 824.5 825 825.5 826 826.5 827 827.5 828 828.5 829 829.5 830 830.5 831 831.5 832 832.5 833 833.5 834 834.5 835 835.5 836 836.5 837 837.5 838 838.5 839 839.5 840 840.5 841 841.5 842 842.5 843 843.5 844 844.5 845 845.5 846 846.5 847 847.5 848 848.5 849 849.5 850 850.5 851 851.5 852 852.5 853 853.5 854 854.5 855 855.5 856 856.5 857 857.5 858 858.5 859 859.5 860 860.5 861 861.5 862 862.5 863 863.5 864 864.5 865 865.5 866 866.5 867 867.5 868 868.5 869 869.5 870 870.5 871 871.5 872 872.5 873 873.5 874 874.5 875 875.5 876 876.5 877 877.5 878 878.5 879 879.5 880 880.5 881 881.5 882 882.5 883 883.5 884 884.5 885 885.5 886 886.5 887 887.5 888 888.5 889 889.5 890 890.5 891 891.5 892 892.5 893 893.5 894 894.5 895 895.5 896 896.5 897 897.5 898 898.5 899 899.5 900 900.5 901 901.5 902 902.5 903 903.5 904 904.5 905 905.5 906 906.5 907 907.5 908 908.5 909 909.5 910 910.5 911 911.5 912 912.5 913 913.5 914 914.5 915 915.5 916 916.5 917 917.5 918 918.5 919 919.5 920 920.5 921 921.5 922 922.5 923 923.5 924 924.5 925 925.5 926 926.5 927 927.5 928 928.5 929 929.5 930 930.5 931 931.5 932 932.5 933 933.5 934 934.5 935 935.5 936 936.5 937 937.5 938 938.5 939 939.5 940 940.5 941 941.5 942 942.5 943 943.5 944 944.5 945 945.5 946 946.5 947 947.5 948 948.5 949 949.5 950 950.5 951 951.5 952 952.5 953 953.5 954 954.5 955 955.5 956 956.5 957 957.5 958 958.5 959 959.5 960 960.5 961 961.5 962 962.5 963 963.5 964 964.5 965 965.5 966 966.5 967 967.5 968 968.5 969 969.5 970 970.5 971 971.5 972 972.5 973 973.5 974 974.5 975 975.5 976 976.5 977 977.5 978 978.5 979 979.5 980 980.5 981 981.5 982 982.5 983 983.5 984 984.5 985 985.5 986 986.5 987 987.5 988 988.5 989 989.5 990 990.5 991 991.5 992 992.5 993 993.5 994 994.5 995 995.5 996 996.5 997 997.5 998 998.5 999 999.5 1000 1000.5 1001 1001.5 1002 1002.5 1003 1003.5 1004 1004.5 1005 1005.5 1006 1006.5 1007 1007.5 1008 1008.5 1009 1009.5 1010 1010.5 1011 1011.5 1012 1012.5 1013 1013.5 1014 1014.5 1015 1015.5 1016 1016.5 1017 1017.5 1018 1018.5 1019 1019.5 1020 1020.5 1021 1021.5 1022 1022.5 1023 1023.5 1024 1024.5 1025 1025.5 1026 1026.5 1027 1027.5 10

plies only where the second heating operation is conducted before the yarn is woven or knitted into fabrics.

It is a feature of the invention that it permits the use of elasticized yarns, and even of elasticized monofilament yarns without plying or similar measures in the manufacture of knit fabrics. This has been previously impossible, because prior art processes are incapable of producing a stable, elasticized, monofilament yarn substantially free of torsional stresses. Knit fabrics formed from non-torsionally stressed yarns according to this invention can be readily distinguished from fabrics formed from conventional elasticized yarns by the loop configuration in the untensioned fabric and by loop behavior upon contraction of the fabric. If one examines a knit fabric formed from elasticized yarns made according to this invention without being torsionally stressed to a high degree, it will be found, when the fabric is stretched to the maximum of its elasticity, that it has a generally normal appearance as if it were made from plain yarns, except that there may be some variation in the size of the interlocking loops of the fabric. When, however, the tension is relaxed and the fabric is allowed to contract in surface area, it will be noticed that a number of things occur. In the first instance, the loops bow and cup so that the previously flat faces of the loops become arcuate and the individual loops no longer lie in a single plane. In a properly finished fabric formed from a well elasticized sample of yarn, the bowing of the loops is frequently so pronounced that in most instances the previously flat face of the loop or, in other words, the surface generally defined by the yarn in the periphery of the loop, is bowed through an arc of from 60 to 180°. Bowing of the loops tends to be especially pronounced near the base or, in other words, the open part of the loop, but is also generally quite apparent near the top of the loop. Secondly, the loop tends to close so that there is a smaller opening at the base of the loop and the yarn forming the loop extends through a greater arc. In some fabrics a portion of the loops will close completely, and in most well elasticized fabrics the yarn in forming the loop will extend through an arc of at least about 270° to 300° when the fabric is completely relaxed. A third change noticeable in many instances and particularly in fabrics knit from monofilament yarns, is that the loops become canted with respect to one another so that they are randomly positioned with respect to the plane of the fabric. The random positioning of the loops with respect to the plane of the fabric is a result of the non-torque elasticization procedure of the invention and does not result in a tendency for the courses of the fabric to become skewed with respect to the wales thereof. High torque elasticized yarns must either be plied or knit "double carrier" with alternating courses or groups of courses of S and Z yarn to prevent or minimize skewing.

A phenomenon which is observed as a result of the above-described elasticizing process is the imparting to the yarn of latent stresses or, in other words, stresses that do not make themselves immediately apparent by changing the linear configuration of the yarn when the tension on the yarn is relaxed. This phenomenon is, of course, quite desirable since it is the release of these stresses during the second heating operation, referred to above, that causes the yarn to develop its full elastic nature and while the exact mechanism involved in the creation of these stresses has not been fully determined, it is known that the stresses are not torsional in nature. For lack of a better phrase, the stresses are referred to as "differential longitudinal stresses" since their potential action is to cause a differential lengthening or shortening of one cross sectional area of the fiber. While their exact nature is not fully understood, the factors which contribute to the creation of these stresses have been accurately determined and will be discussed in subsequent paragraphs.

The yarn to be elasticized according to the new process

of this invention can satisfactorily comprise any continuous filamentary strand composed of an organic, hydrophobic, thermoplastic fiber material; however, nylon yarns such as those formed from the reaction product of hexamethylene diamine and adipic acid or from polymers of caprolactam, are preferred since they can be processed with fewer precautions, are operative through a wider range of conditions and give a higher degree of elasticization than other types of yarn. The invention can, however, also be employed with polyester yarns, such as those prepared from a reaction product of ethylene glycol and terephthalic acid and sold under the name of "Dacron," and under certain conditions, the invention can be employed for the elasticization of polyacrylic fibers formed by the polymerization of acrylonitrile or by the co-polymerization of acrylonitrile with a minor amount of another polymeric monomer. Esters of cellulose, such as cellulose triacetate or cellulose diacetate, are also satisfactory in some instances and a suitable material of this type is available under the trade name of "Arnel." Some yarns give difficulty not so much because of their chemical composition or inherent physical properties but because of their cross sectional configuration. For example, an acrylic fiber sold under the name of "Orlon" has a cross sectional shape resembling the silhouette of a dumbbell and is very difficult to elasticize by the process of this invention. Yarns wherein the filaments have a generally circular cross section and a smooth surface are most readily employed and give the most satisfactory results.

The denier and filament size of the yarn to be processed may vary within wide limits and almost any of the commercially available yarns within the previously specified class can be satisfactorily employed. As an illustration of the wide range of denier and filament sizes which can be employed, excellent results have been obtained by employing nylon yarns of the following descriptions: 15 denier monofilament; 12 denier 4 filament; 100 denier 34 filament; 70 denier 34 filament; 200 denier 34 filaments; 400 denier 68 filament; and 800 denier 51 filament. Under suitable conditions the denier per filament can range from 1 to 20 and the total denier can readily be as high as 2000 or more. For example, excellent results in preparing a nylon yarn for use in the rug industry have been achieved by processing a filamentary nylon strand having a total denier of approximately 2,000 in the manner previously described.

Reference will now be made to the accompanying drawings in which

FIGURE 1 is a schematic view in perspective of apparatus suitable for performing the first step of the process of this invention.

FIGURE 2 is an enlarged view in perspective of a knit fabric according to the invention.

With reference to FIGURE 1 of the drawings, there is illustrated a pair of yarn supply means 10 and 11 mounted on a suitable frame or support member, not illustrated. Yarn ends, indicated by the reference numerals 12 and 13, are led from supply packages 10 and 11 through a pair of guide eyes 14 and 15, about a pair of tension regulating devices 18 and 19 and then to a blade assembly generally indicated by the reference numeral 20. The tension regulating devices 18 and 19 serve the dual purposes of removing the fluctuations in tension resulting from the removal of the yarn from the supply packages 10 and 11 and of supplying the yarn ends to the blade assembly 20 at a proper tension, while the guides 14 and 15 are for the purpose of removing the yarn from the yarn supply packages 10 and 11 as smoothly as possible. From the blade assembly 20, which will be subsequently described in greater detail, the yarn ends are drawn through a portion of the yarn path at 21 having a relatively great radius of curvature, shown in FIGURE 1 as a straight line which would provide the maximum change in curvature and therefore is ordinarily preferred, and are then brought together and passed through a guide 22 to a pair of driven rolls

23. The two yarn ends are then passed through a guide 24 and to a conventional ring and spindle array generally indicated by the reference numeral 25.

The blade assembly, generally indicated by the reference numeral 20, is here illustrated as comprising an arcuate heater strip 30, preferably formed of stainless steel or the like, which has been bent to a radius of about 4 inches in order to present a slightly curved surface to the yarn. The resistance heater strip 30 is adapted to be heated by means of an electric current passed therethrough and is connected by a pair of electrical conductors 31 and 32 to a variable transformer 33 which is supplied with power from any suitable source, not illustrated, through leads 34 and 35. Mounted on the heater strip 30 by means of a holder 38 is a blade member 39 here illustrated as a common razor blade of a type which is commercially available under a number of trade names such as Schick, Gem, etc. The acuate edge 40 of the blade extends beyond the rear edge of the heater strip 30 a short distance so that the yarn ends 12 and 13 pass in contact with the underside of the heater strip and over the edge of blade 39 in an angular path with the edge 40 of blade 39 positioned at the apex of the angular path.

In operation, yarn ends 12 and 13 are threaded through the apparatus in the manner previously described to rolls 23 and the rolls placed in operation so that both yarn ends can be passed together through guide 24 to the spindle array 25. Before further operation of the rolls 23, the adjustable transformer 33 should be set to give sufficient energy to heater element 30 so that it is heated to the desired temperature. With the heater element 30 at the desired temperature and with the apparatus properly threaded, the rolls 23 and the spindle array 25 are placed in operation and thereafter the apparatus requires no further attention unless an end breaks or a yarn supply becomes depleted. By this arrangement two single ends are processed to give them a potentially elastic nature while plying them together to form a two-ply yarn. It will be understood, however, that the yarn ends can be collected singly if desired and that conventional apparatus which does not impart a twist to the yarn can be employed for the collection thereof.

It will be readily apparent to those skilled in the art that apparatus of the type described can readily be constructed by modification of a conventional spinning or twister frame. In either instance all that need be added is the blade assembly 20, the tension devices 18 and 19 and in some instances the guide member 22. In the case of a twister frame, the rolls 23 can constitute the conventional yarn feed means and in the case of a spinning frame the rolls 23 can constitute the delivery pair of the drawing rolls. It will also be apparent that a single heater strip of considerable length can serve a multiplicity of blades spaced at selected intervals corresponding to each position of the frame. In such an arrangement it is usually desirable for the heating element to be insulated, for example, with foam glass insulation, between the various blade positions to reduce the heat loss.

In the type of apparatus described, the yarn is forced through an abrupt change of direction by passing the same over an acuate edge and while this is presently the most convenient method of accomplishing the desired result, it will be apparent that the yarn may be caused to undergo the required abrupt change of direction in other ways.

With particular reference to FIGURE 2 of the drawings, there is illustrated a knit fabric according to this invention formed from monofilament yarn. For ease of illustration the fabric is shown stretched to an extent short of the maximum although it will be understood that the distinguishing characteristics of the fabric are most pronounced when the fabric is in a completely untensioned condition. Canting of the loops with respect to each other and with respect to the plane of the fabric is illustrated by the loops indicated by the reference numerals 50 and 51. This characteristic is among the first to dis-

pear upon stretching of the fabric and as illustrated in the drawings, the loops have been, to a large extent, drawn into the plane of the fabric. The closed nature of the loops is illustrated, for example at 52, and it will be noticed that a majority of the other loops are more nearly closed than might be expected in a conventional knit fabric although the loops have, in most instances, been opened to some extent by stretching of the fabric. Bowing of the loops is clearly evident, for example at 53. This is presently believed to be perhaps the most important characteristic, as far as the elasticity of the fabric is concerned, and is generally the last to disappear as the fabric is stretched.

Although the apparatus for producing yarn containing latent differential stresses is relatively simple, there are several variables which affect the nature of the yarn produced. For example, the radius of curvature of the blade edge, the tension in the strand of yarn as it is passed over the blade, the temperature of the heater element, the rate of cooling of the yarn after it passes the acuate edge and the linear velocity of the yarn can all have their effect upon the nature of the yarn produced and in subsequent paragraphs operative and optimum limits will be set forth for all such variables.

25. The radius of curvature of the acuate edge can vary within reasonably wide limits but is preferably as small as possible without severing the yarn. The smallest possible radius of curvature of the blade in turn depends upon the nature of the yarn being passed over the edge, 30 the size of the filaments in the yarn and upon the texture of the material from which the blade is formed. With a blade formed from a finely grained material, it is possible for the radius of curvature of the edge to be as small as one or two microns when running nylon yarn 35 composed of filaments of about 2 denier or less, but with larger filaments or with other types of yarn, the radius of curvature of the edge should generally be at least about 3 to 6 microns. Even with nylon yarns composed of very small filaments, it is frequently necessary that the radius 40 of curvature be as much as 4 or 5 microns in order for satisfactory results to be obtained if the blade is formed from a coarse textured material. A new razor blade of the blue steel variety generally has a radius of curvature in the vicinity of 1 or 2 microns, but this material is 45 so coarse textured that it is generally necessary for the edge to be smoothed very slightly for best results and this can be accomplished by rubbing the blade a few strokes over a finely abrasive material such as crocus cloth or by polishing the edge with a material such as jeweler's rouge. Stainless steel razor blades, because of 50 their finer texture, can frequently be employed as they are received from the manufacturer, although it is generally preferable, even when processing nylon, to also polish the edges of these blades very slightly to thereby 55 reduce the number of ends down.

55. The maximum radius of curvature of the acuate edge depends primarily upon the size of the yarn filaments being passed thereover, but will also vary to some extent with the chemical nature of the yarn being employed. 60. However, with any type of yarn, it is a general rule that the radius of curvature should be no more than about 1 to 4 times the diameter of the yarn. For example, when using 70 denier 34 filament nylon a good degree of elasticization is generally obtained, only if the radius of curvature of the angular portion of the yarn path is less than about 30 microns, but with a yarn having large filaments, such as 15 denier monofilament nylon, a blade having an edge with a radius of curvature as great as about 70 to 150 microns can sometimes be employed with 65 good results. Even in the latter instance, however, an edge with a radius of curvature less than about 30 microns generally gives the greatest degree of elasticization.

70. Nylon yarn can be passed over the acuate edge in a dry unlubricated condition, but all other yarns generally require the use of a lubricating oil for completely satis-

factory results, and, even with nylon, better results can be achieved by lubricating the yarn prior to its passage over the acuate edge. In the case of multi-filament nylon yarns, it has been found advantageous to employ a lubricating agent which at least partially vaporizes at the temperature of the heater element and while the exact reason for this is not known it is believed that the vaporization of the lubricant results in better heat transfer among the various filaments. In the case of other types of yarn, it is generally preferable to employ a lubricating agent which vaporizes only to an inappreciable extent at the temperature of the heater strip since the yarn needs to be fully lubricated at the time it is passed over the acuate edge or else breakage might occur. In the case of nylon yarns, the preferred lubricating agent has been found to be a low viscosity mineral oil such as that sold under the trademark of "Esso Mentor 20A." In the case of other yarns, the preferred lubricant has been found to be one with a low viscosity and a high flash point and one which can be readily removed from the treated yarn. Sorbitan trioleate is an example of a material which is generally satisfactory. The lubricant can be applied by means of a felt wick, by means of capillary action or by any other means generally used in the textile industry for the application of lubricants to yarns.

The angle of approach and the angle of departure of the yarn to the blade may also vary within wide limits, although the total of these two angles should be less than about  $120^\circ$  and preferably less than about  $100^\circ$ . It is generally advantageous to make the angle of approach relatively large, for example from  $30^\circ$  to  $100^\circ$ , so that the blade is displaced from the heater element and is, therefore, at a lower temperature. On the other hand, it is generally advantageous that the angle of departure be less than about  $50^\circ$  and preferably as small as the grind of the acuate edge will permit. When the angle of approach is relatively large, better than average results can be achieved by allowing the yarn to follow the surface of the blade across its entire width after the yarn passes over the acuate edge. The exact reason or reasons for this are not known with certainty, but it is known that the yarn should preferably be cooled as soon and as rapidly as possible after its contact with the acuate edge, and it is believed that contact across the width of the blade results in a more rapid dissipation of heat from the yarn than is achieved by simply air cooling the yarn as it travels from the acuate edge. If desired, various expedients can be employed to retain the blade at a temperature appreciably below that of the heater element. For example, the blade can be isolated from the heater element by means of heat resistant insulation or a cooling medium can be circulated in contact with the blade to retain it at any desired temperature. While satisfactory results have been achieved with the blade at a temperature equal to that of the heater element, a very marked improvement can be achieved by retaining the blade at a temperature of at least about  $20^\circ$  to  $50^\circ$  F. lower than that of the heater element and preferably at a temperature of at least about  $150$  to  $250^\circ$  below the temperature of the heater element.

The tension in the yarn passing over the blade is another important factor and this variable must be maintained within specified limits to obtain maximum elasticity. Tension measurements are made on the yarn immediately after it leaves the blade edge since it has been found that under near optimum conditions tension in the yarn before it reaches the heating means is too low to be accurately measured. Operative limits for the tension in the yarn following its contact with the acuate edge vary depending upon a number of factors including the temperature of the yarn and the type of yarn being employed but as a general rule, the operative range extends from about .05 gram per denier to approximately 1 gram per denier with the preferred range being from about .1 to .4 gram per denier. The optimum tension will not only vary

with the temperature of the yarn and the yarn composition but also appears to vary slightly with yarns of substantially the same composition made by different manufacturers or even for different lots of yarn made by the same manufacturer. By carefully controlled tests it has been determined that the optimum tension for du Pont type 200 at a temperature of from about  $220$  to  $360^\circ$  F. at the acuate edge is generally from about 0.15 to 0.28 gram per denier.

The linear velocity of the yarn over the blade may also vary within wide limits depending upon the temperature of the heater element, the distance through which the yarn is in contact with the heater element, the distance of the heater element from the edge of the blade and the type of yarn being passed over the blade. It is important that the yarn velocity be such that the yarn accumulates sufficient heat to be at the proper temperature at the moment it contacts the acuate edge and it will be apparent that the yarn velocity required to accomplish this result will vary with the above factors. In other words, with the yarn in contact with the heater element for a given distance and with the heater element at a given temperature, it will take an appreciably longer period of contact for a 70 or 100 denier yarn to be heated than will be required for a 15 or 7 denier yarn, so that a lower yarn velocity must be employed with larger yarn. Likewise, if the acuate edge is too far from the heater element, there is a tendency for the yarn to cool between the heater element and the acuate edge, and it will be apparent that a smaller yarn will cool more rapidly than a larger yarn so that a higher linear yarn velocity must be employed in the first instance. It should also be mentioned that in some instances the average temperature of the heater element may be above the melting temperature of the yarn, and in these instances the linear velocity of the yarn must be sufficiently high to prevent the yarn from melting. As a general rule it may be stated that the operable range for the linear velocity of the yarn over the heater element and acuate edge is from about 1 to 2,000 feet per minute or even higher with the preferred range at present being from 200 to 400 feet per minute.

Although the distance of the acuate edge from the heater element may vary within reasonably wide limits and may be as much as two inches or more, as a general rule it is preferred that the acuate edge be placed as close to the heater element as is possible without actual contact therewith. By placing the acuate edge as close to the heater element as possible, it is only necessary to heat the yarn to substantially that temperature at which it is desired that the yarn contact the acuate edge, whereas if the heater element is removed from the acuate edge, it is necessary that the yarn be heated sufficiently above the temperature at which it is desired that it contact the acuate edge to compensate for the cooling of the yarn that occurs during its passage from the heater element to the edge. Heating the yarn above the optimum temperature for contact with the acuate edge is generally undesirable, since nearly all yarns are weakened to some extent by heat and since temperature control is thereby made more difficult.

The distance over which the yarn is in contact with the heater element should, for optimum results, be as great as is possible without resulting in an undesirably high tension in the yarn. It will be apparent that the greater the distance that the yarn is in contact with heater element, the greater will be the area of contact and the higher will be the tension required to transport the yarn, but under some conditions it has been found that the yarn may be maintained in contact with a heater element for as much as 12 to 20 inches or more without introducing excess tension. A heater element which results in the yarn being in contact therewith for a distance of approximately 1 to 10 inches is presently preferred in most instances since this length of contact is adequate for most small yarns (i.e. below 100 denier) at yarn velocities below

about 400 to 1000 feet per minute. With yarn velocities in excess of 400 to 1000 feet per minute or with high denier yarns, it is generally preferable that the yarn be retained in contact with the heater element for a greater distance and under these conditions, a heater element having a width of 10 to 12 inches or more is frequently advantageous. No minimum distance for retaining the yarn in contact with the heater element can be specified since by employing low yarn velocities, an almost infinitesimal distance can be satisfactory and good results have been achieved by employing only the edge of the blade itself as a heater element. There is, however, generally no advantage in attempting to employ a heater element such that the yarn is retained in contact therewith for less than about  $\frac{1}{4}$  inch and as previously stated, if higher yarn velocities are to be employed, greater distances of yarn contact should be utilized.

A further factor which need be considered in the production of the latently elasticized yarn is the temperature of the heater element and it will be appreciated that the operative range for this variable depends upon the type of yarn being employed, the linear velocity of the yarn, and the distance for which the yarn is in contact with the heater element. If a moderately high yarn velocity is employed, for example 100 to 1000 feet per minute, and the contact of the yarn with the heater strip is limited to a short distance, for example 1 inch or less, it is possible to obtain satisfactory results with the heater element at an average temperature appreciably higher than the melting point of the yarn. For example, under such conditions operative results can be achieved with nylon yarns with the heater element at a temperature of 500° F. or even higher. On the other hand, if the yarn is maintained in contact with the heater element for a relatively long distance, for example from 3 to 9 inches, it is possible to obtain operative results with the heater element at a temperature as low as about 180° F. with nylon yarn. The optimum temperature for the heater element will, of course, depend upon the type of yarn being employed as well as the other factors considered above, but even with yarns of the same composition, the optimum temperature of the heater element appears to depend upon the filament size in the yarn being employed. For example, with the yarn in contact with the heater element for a distance of approximately 3 inches and with a yarn velocity of 120 feet per minute, an operating temperature of from about 320 to 360° F. has been found to be optimum for processing 15 denier monofilament nylon (type 66, semidull) while a temperature of from about 330 to 380° F. for the heating element appears to be optimum when processing 30 denier 10 filament nylon. In other words, since the optimum temperature of the heater element will vary slightly depending upon many factors, it is generally advantageous to conduct a series of tests to determine the optimum temperature for the heater element for each particular set of conditions encountered.

The temperature of the heater element has been emphasized since under normal operating conditions the exact temperature of the yarn passing over the acuate edge is difficult to measure, but it will be apparent that the really important consideration is the temperature of the yarn as it contacts the blade edge. With all yarns of a given construction and chemical composition there is a well defined operative temperature range for the yarn at this point and some of the values for the heater element temperature set forth above are only made necessary or possible because of other variables. Although the exact lower operative limit for any given type of yarn will vary slightly, it can be stated as a general rule that the lower limit is that temperature which is sufficient to at least largely relax the stresses normally present in the yarn or in other words, sufficient to relieve the yarn of a large part of the residual shrinkage present therein. The yarn as it passes over the heating element is generally under such a low tension that it readily contracts and a tem-

perature which will result in the yarn contracting to the extent that it has a residual shrinkage of no more than about 1 to 5% at the time of its contact with the acuate edge is generally sufficient to result in operative conditions. For nylon yarns, the lower operative limit will vary from about 180° F. for type 6, 15 denier monofilament up to approximately 240° F. for nylon yarns which are very difficult to elasticize. For other types of yarns the operative lower limit will vary from about 190° F. to 300° F. The upper operative temperature for the yarn as it contacts the acuate edge is generally that temperature at which the yarn begins to display a tendency to stick to surfaces with which it is in contact, or as it is called in trade and scientific publications, the "sticking temperature" of the yarn. The optimum temperature for the thermoplastic strand as it contacts the acuate edge will vary with a number of factors including filament size and chemical composition and generally must be empirically determined for each specific yarn. For example, by actual operation it has been found that the optimum temperature for du Pont type 200 nylon, 15 denier monofilament yarn is about 320 to 340° F., while the optimum temperature for type 200 nylon, 70 denier, 34 filament yarn is about 340 to 370° F. A simple test, which has been found to be of some value in estimating an optimum temperature for most types of yarn, comprises measuring the tension developed in a given length of the yarn as the temperature is raised. As the temperature of the yarn is increased, a point is reached where the tension developed in the yarn falls off rapidly and this point is generally a near optimum for passing this particular type of yarn to the acuate edge.

While it is not absolutely necessary that the thermoplastic end of yarn be cooled after its contact with the acuate edge, cooling the yarn is generally more convenient than retaining it at an elevated temperature and, in most instances, rapidly lowering the temperature of the yarn 100 to 200° F. or more results in a better product. As a general rule the temperature of the yarn should be reduced until it is at least 20 to 80° F. below the minimum temperature at which the yarn may satisfactorily be passed through the acutely angular portion of the yarn path. For example, with nylon the temperature of the yarn should be lowered at least to about 160° F. One convenient method of cooling the yarn comprises subjecting the yarn, immediately subsequent to its contact with the acuate edge, to the atmosphere so that the yarn end is cooled by air currents. Still another and generally more satisfactory method comprises passing the yarn into contact with a cold metallic surface such as the side of the blade when the blade is so positioned that it is not heated to a high temperature by the heating means. Other means of cooling the yarn end after its contact with the acuate edge will readily suggest themselves to those skilled in the art.

The radius of curvature of the portion of the yarn path immediately following the point where the yarn passes about the acuate edge and wherein the yarn is subjected to cooling conditions, should be relatively large as compared to the radius of curvature of the acutely curved portion of the yarn path. This is most conveniently achieved by passing the yarn through a straight line path, as shown in FIGURE 1, although as stated previously a definitely curved path is acceptable if its radius of curvature is considerably greater than that at the blade edge. It is believed that the lack of liveliness in the latently elasticized yarn is at least partially a result of passing the yarn from the highly curved portion of the path into a portion of the path having a relatively large radius of curvature. As a general rule, the radius of curvature of the portion of the path immediately following the acutely curved portion should be no less than about 600 microns and should preferably be at least one inch. The length of this portion of the path need not be great and adequate cooling of the yarn can generally be accomplished in  $\frac{1}{8}$

inch or less, although a length of one inch or more is generally preferred.

To transform the latently elasticized yarn to a fully elasticized condition, it is necessary to positionally relax the stresses created in the yarn as a result of its being passed through the angular path in a heated condition.

If the full elastic nature of the latently elasticized yarn is to be developed before the yarn is formed into fabrics, the heating can be conducted by overfeeding a single end of the potentially elastic yarn into a heated fluid or into contact with a heated surface so that the yarn is allowed to coil freely at the time its temperature is elevated. A high temperature is not required and satisfactory results can generally be obtained if the yarn is heated to a temperature of only about 120° F. although a temperature of from about 140 to 400° F. is generally preferred. Care should be exercised to insure that the yarn at the time it is heated is under as little tension as possible, and if the tension in the yarn is allowed to rise above about .004 to .01 gm./denier, good elasticizing may not be obtained. If the tension in the yarn is at a proper level, the yarn assumes a highly convoluted linear configuration almost immediately so that the heating need not be continued for more than 1 or 2 seconds. As an alternative to the above procedure, the yarn can be formed into skeins and the skeins immersed in a hot liquid or passed through a heated chamber to result in the yarn developing its full elastic nature. When the yarn is fully elasticized by either of these procedures before its formation into fabric, no special manipulations of the woven or knitted fabrics are required, although it is generally advantageous to weave or knit the yarn in a loose manner so that upon relaxation of the tension necessary for weaving or knitting, the yarn is free to curl or kink to provide the desired effect.

Having thus described my invention, what I desire to claim and secure by Letters Patent is:

1. A method of crimping a continuous filament thermoplastic yarn which comprises the steps of continuously passing said yarn in an acutely angular path such that at the apex of the acute angle in the yarn path, the yarn is conformed to an arch having a mean radius of curvature of from 1 to 150 microns, continuously heating the yarn in one segment of the yarn path so that at least the segment of the yarn transiently disposed at said apex is at a temperature sufficient to plasticize but insufficient to melt the yarn and thereafter heating the yarn before the yarn is formed into fabric to a temperature of at least 120° F. while it is under insufficient tension to prevent the same from contracting in length.

2. A method of crimping a continuous filament thermoplastic yarn which comprises continuously passing said yarn through a heating zone maintained at a temperature sufficient to plasticize but insufficient to melt the yarn,

immediately thereafter passing the heated yarn in an angular path over the sharp edge of a blade while under tension, said edge being disposed at the apex of the acute angle formed between the path of delivery to, and the path of withdrawal of the yarn from said edge and thereafter heating the yarn before the yarn is formed into fabric to a temperature of at least 120° F. while it is under insufficient tension to prevent the same from contracting in length.

10 3. A method according to claim 1 wherein the heating operation is conducted by forming the yarn into skeins and subjecting the skein to the action of a heated fluid.

4. A method according to claim 1 wherein the heating operation is conducted on a running length of yarn.

15 5. A method for processing a continuous filament thermoplastic yarn, the filaments of which are substantially free of torsional stresses and which, when relaxed, contain at least 5 loops per inch of from about 1 to 3 millimeters in diameter, about half of which are in one direction, 20 and the remaining half are in the opposite direction, and which contain latent differential longitudinal stresses sufficient to produce, when the yarn is heated in an untensioned condition, loops about half of which are in one direction and the remaining half in the opposite direction, 25 which have an average diameter of from 0.2 to 0.9 millimeter and which are so closely spaced as to form a substantially closed helix between reversal points, said method comprising heating the yarn before the yarn is formed into fabric to a temperature of at least 120° F. by over- 30 feeding the yarn at a tension of less than 0.01 gm./denier into contact with a heated surface for less than two seconds so that the yarn is allowed to coil freely at the time its temperature is elevated.

6. The method of claim 5 wherein the yarn is heated 35 to a temperature of from about 140 to 400° F.

7. The method of claim 6 wherein the yarn is nylon.

**References Cited in the file of this patent**

UNITED STATES PATENTS

|    |           |                 |       |               |
|----|-----------|-----------------|-------|---------------|
| 40 | 2,277,782 | Rugeley         | ----- | Mar. 31, 1942 |
|    | 2,369,395 | Heymann         | ----- | Feb. 13, 1945 |
|    | 2,379,824 | Mummery         | ----- | July 3, 1945  |
|    | 2,435,891 | Lodge           | ----- | Feb. 10, 1948 |
| 45 | 2,525,543 | Guttman et al.  | ----- | Oct. 10, 1950 |
|    | 2,536,163 | Field et al.    | ----- | Jan. 2, 1951  |
|    | 2,669,001 | Keen            | ----- | Feb. 16, 1954 |
|    | 2,685,120 | Brant           | ----- | Aug. 3, 1954  |
|    | 2,875,502 | Matthews et al. | ----- | Mar. 3, 1959  |
| 50 | 2,919,534 | Bolinger et al. | ----- | Jan. 5, 1960  |

## FOREIGN PATENTS

558,297 Great Britain ----- Dec. 30, 1943  
164,127 Australia ----- July 15, 1955